

## UNITED STATES PATENT OFFICE

2,025,803

OXIDIZED PRODUCT OF WATER-INSOLUBLE  
HYDROXYLATED FATTY ACIDS.

Melvin De Groot, St. Louis, and Bernhard Keiser,  
Webster Groves, Mo., assignors to Tretolite  
Company, Webster Groves, Mo., a corporation  
of Missouri

No Drawing. Application November 12, 1934,  
Serial No. 752,721

4 Claims. (Cl. 87—12)

This invention relates to a new oxidized fatty body and to a method of producing the same.

One object of our invention is to provide a new material, composition of matter, or chemical compound that is capable of various industrial uses, but particularly, adapted for use as a treating agent or demulsifying agent in the resolution of petroleum emulsions of the water-in-oil type. Said new material, composition of matter, or chemical compound may be properly described as an oxidation product or products derived by blowing the hydrolytic products (hydroxylated fatty acids), obtained by subjecting a linseed oil-type fatty acid sulfation mass to hydrolysis. These products are referred to as oxidation products because they are somewhat similar to conventional oxidized or blown oils, and are obtained by oxidizing or blowing certain hydroxylated fatty acids, hereinafter described, by means of air or oxygen. The fatty products or hydroxylated fatty acids which are subjected to oxidation, are derived by the hydrolysis of the sulfation mass obtained by treating linseed oil-type fatty acids, such as linseed oil fatty acids or perilla oil fatty acids, with sulfuric acid, at approximately 35° to 54° C. Linseed oil fatty acids or perilla oil fatty acids are obtained from linseed oil or from perilla oil, respectively, by the usual method of fat splitting, such as a Twitchell process.

It is customary to oxidize or blow certain non-drying oils, such as castor oil or red oil, by means of dry or moist air or oxygen. Castor oil is used most frequently for this purpose. Similarly, the said procedure is employed to blow semi-drying oils such as cottonseed oil. The products so obtained have found use in various arts in the past, such as in the manufacture of lubricants, or as plasticizers in the manufacture of artificial leather, etc. Blown or oxidized castor oil has found use in the demulsification of crude oil.

Oxidation or blowing of a true drying oil such as linseed oil or perilla oil yields a leathery mass or a product such as linoleum. It is unsatisfactory to attempt to produce a blown oil solely from true drying oils. Statements have appeared in the literature that blown oils can be produced from linseed oil and the like. Blown oils, if produced from linseed oil, at the most, represent nothing more than an incipient oxidation, and do not represent a blown oil which is basically changed in chemical characteristics in the manner corresponding to the change which occurs in blown castor oil. Reference is made to U. S. Patent No. 1,929,399, to Fuchs, dated October 3,

1933, in which the chemical characteristics of a truly blown castor oil are indicated.

The same chemical activity which results in a stringy or leathery product, of relatively worthless properties, when one attempts to drastically blow or oxidize linseed oil, is also responsible for the inability to sulfonate or sulfate linseed oil so as to yield an acceptable and valuable sulfonation product. It is impractical to treat linseed oil with sulfuric acid so as to produce a Turkey red oil substitute suitable for the purposes for which Turkey red oil is ordinarily employed.

In U. S. Patent No. 1,745,221, to Bernhard Keiser, dated January 28, 1930, there is disclosed a method of making a hydroxylated sulfation product from linseed oil or perilla oil, by sulfation of the fatty acids derived from the glycerides. Briefly stated, it is disclosed in that patent that the fatty acids of these true drying oils, for some unknown reason, can be readily sulfonated or sulfated so as to yield a product akin to Turkey red oil. The process there disclosed contemplates the converting of linseed oil or perilla oil into the fatty acids by means of the well known Twitchell process, or any other acceptable process conventionally employed for fat splitting. The fatty acids thus obtained are sulfated or sulfonated with 64° Baumé sulfuric acid, at a temperature not to exceed 54° C.

In the method employed to produce our new material or composition of matter, we follow the same procedure as disclosed in said Keiser patent, so far as the sulfation goes. After the sulfation of linseed oil fatty acids, for example, with approximately 50% by weight of 64° Baumé sulfuric acid at not over 54° C., we wash the product with an approximately equal weight of water and allow the mixture to stand until two layers form. The lower layer is withdrawn and discarded. This washing process may be repeated, if desired. The upper fatty layer, consisting largely of linseed oil fatty acid sulfates, perhaps already partially hydrolyzed, is water-soluble in a 10% solution. It is diluted with an approximately equal volume of water, and then treated with live steam until it is no longer water-soluble, and until it is substantially free from all combined sulfurtrioxide. This product, so obtained, is the hydrolytic product derived by decomposition of the materials obtained by sulfation of linseed oil fatty acids. For the sake of brevity, we refer to these particular products as the hydroxylated fatty acids. It is to be noted that the expression "hydroxylated fatty acids" refers solely to the products thus obtained by hydrolysis of the sulfation mass ob-

tained by treatment of linseed oil fatty acids or perilla oil fatty acids, with sulfuric acid, under conditions to yield a water-soluble, non-stringy mass. To prevent corrosion, any acidity to 5 methyl orange indicator can be neutralized with a suitable base, such as caustic soda.

We oxidize or blow these hydroxylated fatty acids in the conventional manner with either moist or dry air, or moist or dry oxygen. We 10 prefer to use air with its normal content of moisture. One procedure which we have found suitable is to heat these hydroxylated fatty acids to approximately 150° C., and then blow with air for several hours, possibly as much as fifteen 15 hours, in order to give a heavy bodied fatty product of increased viscosity and increased specific gravity. Such a product is substantially free from any stringiness. The product thus obtained is effective as a demulsifying agent for crude oil 20 emulsions of the water-in-oil type, especially after dilution with a solvent, such as xylene. It is possible that such product may be used advantageously in the arts where blown oils of the conventional type have been found to be of value. 25 It is understood, of course, that in hydrolyzing the sulfation mass previously described, that there may be added a small amount of Twitchell agent or any other material which would hasten the hydrolytic reactions. It is also understood 30 that a certain amount of unsulfonated or non-hydroxylated fatty material may be present in

the sulfation mass, and remain in the finally washed product.

Having thus described our invention, what we claim as new and desire to secure by Letters Patent is:

1. A new composition of matter, consisting of the oxidized product derived by blowing until substantial oxidation takes place, water-insoluble hydroxylated fatty acids, obtained by the hydrolytic decomposition of linseed oil type fatty acid 10 sulfates.

2. A new composition of matter, consisting of the oxidized product derived by flowing until substantial oxidation takes place, water-insoluble hydroxylated fatty acids obtained by the hydrolytic 15 decomposition of linseed oil fatty acid sulfates.

3. A method of producing a new composition of matter of the kind described, characterized by blowing until substantial oxidation takes place, 20 water insoluble, hydroxylated fatty acids, obtained by the hydrolytic decomposition of linseed oil type fatty acid sulfates.

4. A method of producing a new composition of matter of the kind described, characterized by 25 blowing until substantial oxidation takes place, water insoluble, hydroxylated fatty acids, obtained by the hydrolytic decomposition of linseed oil fatty acid sulfates.

MELVIN DE GROOTE. 30  
BERNHARD KEISER.